

July 3, 1934.

M. PIER ET AL

1,965,390

PRODUCTION OF VALUABLE LUBRICATING OILS

Filed March 16, 1931

2 Sheets-Sheet 1



INVENTORS  
MATHIAS PIER  
FRIEDRICH CHRISTMANN  
BY  
Hauffel Warland  
ATTORNEYS

July 3, 1934.

M. PIER ET AL

1,965,390

PRODUCTION OF VALUABLE LUBRICATING OILS

Filed March 16, 1931

2 Sheets-Sheet 2



INVENTORS  
MATHIAS PIER  
FRIEDRICH CHRISTMANN  
BY  
Hausfeld Warland  
ATTORNEYS

## UNITED STATES PATENT OFFICE

1,965,390

## PRODUCTION OF VALUABLE LUBRICATING OILS

Mathias Pier, Heidelberg, and Friedrich Christmann, Ludwigshafen-on-the-Rhine, Germany, assignors to I. G. Farbenindustrie Aktiengesellschaft, Frankfort-on-the-Main, Germany

Application March 16, 1931, Serial No. 523,178  
In Germany April 5, 1930

10 Claims. (CL 196—78)

This invention relates to improvements in the manufacture and production of valuable lubricating oils.

It is already known that lubricating oils may be obtained by polymerizing unsaturated hydrocarbons. Frequently, however, for example when employing initial materials comparatively poor in hydrogen, resinous substances are formed, the quality of the lubricating oils thus being considerably impaired.

10 We have now found that excellent lubricating oils are obtained by subjecting unsaturated hydrocarbons to condensation in stages carried out at successively higher temperatures, the condensed products being separated at least before the second stage. In this manner a condensation product which is mainly poor in hydrogen is obtained in the first stage of the polymerization carried out at low temperatures and this is separated, for example, by distillation in vacuo, and in the following stages carried out at successively higher temperatures a lubricating oil rich in hydrogen and of the best quality is obtained. The process according to the present invention is particularly adapted for the production of high quality lubricating oils, from those unsaturated hydrocarbons which by a condensation carried out in one operation would yield only lubricating oils of low quality. The term "condensation" where employed in the present application is also intended to include within its scope "polymerization".

As the initial materials may be mentioned unsaturated hydrocarbons from any source, which are liquid under normal conditions of temperature and pressure. They should have a high iodine value, often exceeding 100 and preferably exceeding 200. The said hydrocarbons may be obtained by the dehydrogenation for example of hydrocarbons of any molecular weight rich in hydrogen, especially paraffinic or naphthenic hydrocarbons, as for example benzenes or middle oils or of petroleum residues, such as petrolatum, or of destructive hydrogenation products of coals, tars, mineral oils and the like or of lubricating oils rich in hydrogen, but of low viscosity, or of synthetically prepared products which have been prepared by the reduction of the oxides of carbon with or without pressure. The dehydrogenation may be effected for example by cracking hydrocarbons, in particular those rich in paraffins and of high molecular weight, as for example paraffin wax, at temperatures below 600° C., preferably in the presence of catalysts such as metals of the 6th group of the periodic system or their

compounds, especially oxides, either alone or in admixture with each other or copper or the like at atmospheric or increased pressure, if desired with the addition of hydrogen. In the cracking a splitting of the carbon chains takes place simultaneously.

The cracking may be carried out in coils or tanks or both. It is particularly advantageous to carry out the cracking in several stages of different pressures. For example, the hydrocarbons may first be cracked under a moderately elevated pressure of about 10 atmospheres, and then under a lower pressure and at a higher temperature. The cracked products obtained are mainly unsaturated hydrocarbons having a high iodine value, preferably above 130, liquid under normal conditions of temperature and pressure, and boiling for the most part between 30° and 300° C. Gaseous olefines such as ethylene, propylene and butylene are also obtained in relatively small amounts. These may also be subjected to the condensation. The dehydrogenation of the said initial materials may also be effected by treatment under dehydrogenating conditions with halogen or halogen-exchanging halogen compounds, if desired in the presence of halogen transmitters, such as iodine, antimony trichloride and the like, the halogen then being split off in the form of its hydrogen compounds. Instead of halogen other substituents such as oxygen or sulphur may be employed.

The dehydrogenated products are then condensed in stages of successively increasing temperatures, usually of below 150° C. and preferably in the presence of condensing agents, such as anhydrous inorganic halides, for example aluminium chloride, zinc chloride, boron fluoride, iron chloride, phosphorus oxychloride, or activated aluminium, sodium, zinc dust or the like.

The successive increase in temperature from stage to stage may be small, as for example 3° or 5° C., but often a considerably greater increase in temperature, as for example from 30° to 70° C. is set up. The condensation carried out in stages may also be effected by varying the condensation agents. It may be advantageous to operate with condensing agents of increasing activity. As a rule the activity of the condensing agent may be said to increase in the following order:—zinc dust, sodium, activated aluminium, iron chloride, boron fluoride, zinc chloride and aluminium chloride. It should, however, be understood that the said order need not necessarily hold good under all conditions. It is also advantageous to carry out the condensation in the presence of

substances of large surface area, such as Florida earth, bleaching earth or silica gel, either alone or together with the condensing agents hereinbefore mentioned or to subject the condensation products to a subsequent treatment. In some cases it is important to carry out the condensation with the addition of compounds which retard the reaction, such as zinc oxide, soda, ammonia and the like. The single stages may also be carried out with the addition of cyclic hydrocarbons, such as naphthalene or mineral coal tar fractions, as for example crude benzol, anthracene oil and the like, as well as aromatic oils which have been obtained by destructive hydrogenation or dehydrogenation, or gaseous olefines, such as cracking gases and the like. The duration of the condensation in each stage depends in part on the concentration of the condensing agent employed. For example when working with an addition of 7 per cent by weight of aluminium chloride the duration of the treatment under certain conditions to produce the degree of condensation desired in the particular stage may be about 0.5 to 5 hours. On the other hand when working under otherwise the same conditions with an addition of 2 per cent by weight of anhydrous aluminium chloride, the duration of the treatment must be 5 to 12 hours. It should of course be understood that the said durations are merely stated in order to illustrate the relative rate of the reaction, and that these may be varied by one skilled in the art depending on the conditions otherwise employed.

In the said condensation in stages the products poorer in hydrogen are usually first condensed, and each subsequent stage then furnishes a lubricating oil richer in hydrogen.

The condensation products formed and separated in the first stage, if they do not already have lubricating properties may be converted by treatment with hydrogen under pressure into products richer in hydrogen which may serve as initial materials for the synthesis of lubricating oils.

The invention will be further explained with reference to the accompanying drawing showing in a somewhat diagrammatic manner an elevation, partly in section, of a plant which is particularly advantageous for carrying into effect the process according to the present invention. The invention is, however, not restricted to the particular arrangement shown in the said drawing.

Referring to this drawing in detail letter *a* denotes a cracking shell heated with hot gases in which a crude lubricating oil rich in hydrogen is cracked at a temperature between 500° and 550° C. The evaporated cracked products pass from *a* into cooler *b* and from thence into the separator *c* from which the gaseous constituents not condensed in *b* are drawn off through pipe *d*. The condensed cracked products are collected in the storing vessel *f* from which they are conveyed by means of pump *g* into a stirring vessel *h* heated with steam. In this vessel *h* the condensation with aluminium chloride introduced at *h*<sub>1</sub> takes place at about 30° C. The contents of vessel *h* are thereupon allowed to flow into vessel *e* in which the condensed hydrocarbon product is separated from the waste aluminium chloride. The heavier aluminium chloride deposits on the conical bottom of vessel *e* from which it may be drawn off through pipe *e*<sub>2</sub>. The condensed hydrocarbon product is removed through pipe *e*<sub>1</sub> mounted on vessel *e* at a medium height.

The condensation product freed from the aluminium chloride is then passed into a stirring vessel *k* and from thence by means of pump *l* into the preheater *m* heated with hot gases. The preheated products are then introduced into the distillation column *n*. In the preheater *m* steam is simultaneously produced which enters the column *n* at *q*. The condensation products freed from lower boiling constituents carried off through pipe *o* are drawn off from column *n* through pipe *p* and then to storage vessel *r*, while the said lower boiling constituents containing benzines and middle oil are passed through a condenser *s* and from thence into the separator *t*. From this separator the uncondensed gases escape through pipe *t*<sub>1</sub> while the condensed products are conveyed by way of stirring vessel *u* and pump *v* into a second stirring vessel *w* in which they are condensed for a second time with aluminium chloride at a higher temperature, for example 100° C. The aluminium chloride is introduced at *w*<sub>1</sub>. After the condensation the contents of vessel *w* are drawn off into vessel *x* in which the separation of the reaction product from the waste aluminium chloride takes place. The aluminium chloride is drawn off from vessel *x* through pipe *x*<sub>2</sub> while the condensation products are removed through pipe *x*<sub>1</sub> mounted on vessel *x* at a medium height.

The following examples will further illustrate the nature of this invention, but the invention is not restricted to these examples. The parts are by weight.

#### Example 1

100 parts of an American petroleum residue (petrolatum) are cracked several times at from 500° to 540° C. In addition to 5 parts of coke and 25 parts of cracking gas, 70 parts of a strongly unsaturated oil having an iodine value of 145 are obtained. This oil is polymerized at from 15° to 30° C. with an addition of 4 parts of aluminium chloride while stirring. After decomposing the aluminium chloride with water, 8 parts of resin are obtained and by distillation 55 parts of a light oil having an iodine value of 120 and a distillation residue of 7 parts of a lubricating oil poor in hydrogen and somewhat resinous and having a steep temperature-viscosity curve are obtained.

The said 55 parts of light unsaturated oil are again polymerized at a temperature of from 30° to 110° C. with an addition of 5 parts of aluminium chloride. In addition to 25 parts of a saturated benzine and a middle oil, 30 parts of a lubricating oil are obtained having a viscosity of 3° Engler at 100° C. and the temperature-viscosity curve of a Pennsylvanian lubricating oil.

#### Example 2

100 kilograms of a producer tar boiling between 200° and 325° C. are stirred in a stirring vessel for 8 hours and at a temperature of 125° C. with a mixture of 1 kilogram of boric acid and 3 kilograms of oxalic acid. After allowing the mixture to cool the liquid is separated from the precipitate and then subjected to distillation. 14.5 kilograms of a lubricating oil is obtained of which 50 per cent have a viscosity of 20° Engler at 50° C. The non-condensed part is treated with 6 kilograms of aluminium chloride at 130° C. After working up 27 kilograms of a lubricating oil are obtained of which 50 per cent consist of a gas machine oil having a viscosity of 12° Engler at 50° C. By the polymerization carried

out in stages the formation of resinous residues is lowered to 12 per cent, whereas when carrying out the condensation in one operation more than 30 per cent of resinous residues are obtained.

*Example 3*

100 kilograms of producer tar boiling between 200° and 325° C. are thoroughly stirred in a stirring vessel at a temperature of about 125° C. for a period of about 8 hours with a mixture of 1 kilogram of boric acid and 3 kilograms of oxalic acid. On cooling, the sediment is separated off and on distillation of the oil, 14.5 kilograms of a lubricating oil are obtained which can be divided up into fractions of different viscosities.

That portion of the initial material which has not yet undergone condensation is treated with 6 kilograms of aluminium chloride at a temperature of about 130° C. and furnishes 27 kilograms of a lubricating oil after being worked up.

What we claim is:—

1. A process for the production of lubricating oils from a liquid hydrocarbon product essentially comprising unsaturated hydrocarbons which comprises subjecting said liquid hydrocarbon product in a first stage to partial chemical condensation to condense mainly the more unsaturated hydrocarbons in the presence of a chemical condensing agent at a temperature at which condensation without substantial cracking takes place to produce a lubricating stock comparatively poor in hydrogen, separating the condensed products from the uncondensed constituents and subjecting the latter in at least one further stage to chemical condensation to produce a lubricating stock richer in hydrogen in the presence of a chemical condensing agent at a temperature at which condensation without substantial cracking takes place, and which is at least 3° C. higher than the temperature used in said first stage, the elevation of the temperature depending on the relative activities of the condensing agents used in the separate stages.

45

2. The process according to the preceding claim in which the initial material is such as would yield a low quality lubricating oil when subjected to chemical condensation in one stage.

3. The process defined in claim 1 in which the unsaturated hydrocarbons contained in the initial material boil between about 30° and about 325° C.

4. The process according to claim 1 in which the initial material boils between about 30° and about 325° C. and possesses an iodine number exceeding 100 and yields a low quality lubricating oil when subjected to chemical condensation in a single stage.

5. The process according to claim 1 in which the initial material is obtained by dehydrogenating a hydrocarbon mixture of high molecular weight and rich in hydrogen.

6. The process according to claim 1 in which the difference between the temperature employed in the second stage and the first stage is between 3° and 70° C.

7. The process according to claim 1 in which a cyclic hydrocarbon is employed in admixture with the material.

8. The process according to claim 1 in which the chemical condensing agent employed in the second stage is different from the chemical condensing agent employed in the first stage.

9. The process according to claim 1 in which the chemical condensing agent employed is anhydrous aluminium chloride.

10. A process for the production of a lubricating oil, which comprises cracking petrolatum at temperatures of between 500° and 540° C., condensing the resulting liquid unsaturated hydrocarbons at a temperature of from 15° to 30° C. with an addition of anhydrous aluminium chloride, distilling off the light unsaturated oil thus obtained as a lubricating oil, and condensing said light unsaturated oil by treatment with anhydrous aluminium chloride, at a temperature of between 30° and 110° C.

MATHIAS PIER.  
FRIEDRICH CHRISTMANN.

120

125

130

135

140

145

150

50

55

60

65

70

75